# EUROPEAN PATENT SPECIFICATION

(11) **EP 0 585 940 B1**
(45) Date of publication and mention of the grant of the patent: **08.07.1998**
(21) Application number: 93114142.8
(22) Date of filing: 03.09.1993
(51) Int. Cl.: C22C 38/00, C22C 38/48, C22C 38/34, C22C 38/14, C22C 38/16, C22C 19/00, H01F 10/00, H01F 10/12

(54) **Alloy with ultrafine crystal grains excellent in corrosion resistance**
Legierung mit ultrafeinen Kristallkörnern und hervorragender Korrosionsbeständigkeit
Alliage à grains cristallins ultrafins à résistance excellente à la corrosion

(30) Priority: 03.09.1992 JP 235467/92
(43) Date of publication of application: 09.03.1994
(73) Proprietor: HITACHI METALS, LTD., Chiyoda-ku, Tokyo (JP)
(72) Inventor: Yoshizawa, Yoshihito, Fukaya-shi, Saitama-ken (JP); Arakawa, Shunsuke, Kumagaya-shi, Saitama-ken (JP); Sugimoto, Katsuhisa, Sendai-shi, Miyagi-ken (JP)
(74) Representative: Beetz & Partner Patentanwälte

(56) References cited:
- EP-A- 0 429 022
- EP-A- 0 430 085
- CHEMICAL ABSTRACTS, vol. 117, no. 12, September 27, 1992, Columbus, Ohio, USA YOSHIZAWA, KATSUTO et al. "Ultrafine-grain iron alloys having asymetric magnetiza- tion curve and their manufacture." page 273, column 1, abstract- -no. 116 030y
- CHEMICAL ABSTRACTS, vol. 117, no. 6, August 10, 1992, Columbus, Ohio, USA CHO, TSUTOMU et al. "Powder manufacture from melt- quenched iron alloy having soft magnetic properties." page 296, column 2, abstract- -no. 53 350e
- CHEMICAL ABSTRACTS, vol. 117, no. 6, August 10, 1992, Columbus, Ohio, USA HASEGAWA, NAOYA et al. "Soft magnetic alloy films." page 880, column 2, abstract- -no. 61 307m
- CHEMICAL ABSTRACTS, vol. 114, no. 22, June 3, 1991, Columbus, Ohio, USA YOSHIZAWA, KATSUTO et al. "Heat treatment in grain refinement of soft magnetic iron alloy." page 277, column 2, abstract- -no. 211 608q
- CHEMICAL ABSTRACTS, vol. 113, no. 26, December 24, 1990, Columbus, Ohio, USA YOSHIZAWA, KATSUTO et al. "Heat-resistant soft magnetic iron alloys." page 239, column 1, abstract- -no. 235 443n
- CHEMICAL ABSTRACTS, vol. 115, no. 22, December 2, 1991, Columbus, Ohio, USA HASEGAWA, NAOYA "Soft magnetic cobalt alloy film." page 989, column 1, abstract- -no. 246 445q
- CHEMICAL ABSTRACTS, vol. 118, no. 12, March 22, 1993, Columbus, Ohio, USA CHEN, GUOJUN "New soft magnetic alloys - ultrafine crystalline alloys: structure and magnetism." page 916, column 1, abstract- -no. 114 955a
- CHEMICAL ABSTRACTS, vol. 116, no. 24, June 15, 1992, Columbus, Ohio, USA YOSHIZAWA, KATSUTO et al. "Ultrafine crystalline alloys having perminvar characteristics." page 820, column 1, abstract- -no. 247 191d

## Description

### BACKGROUND OF THE INVENTION

This invention relates to an ultrafine-crystalline alloy excellent in soft magnetic properties and corrosion resistance.

Silicon steel, Fe-Si alloys, amorphous alloys, etc. are well known as soft magnetic materials, and their important properties are high relative permeability µ and saturation magnetic flux density Bs.

In addition to magnetic properties, corrosion resistance is an important property since these magnetic materials would be used under various circumstances.

However, it had been considered difficult to achieve both high saturation magnetic flux density Bs and high relative permeability µ at a time in the magnetic materials. Fe-based amorphous alloys have, for example, high saturation magnetic flux density Bs, while they are inferior to Co-based amorphous alloys in soft magnetic properties. On the other hand, the Co-based amorphous alloys are excellent in soft magnetic properties, while they do not have sufficient saturation magnetic flux density Bs.

High saturation magnetic flux density Bs and high relative permeability µ had conventionally been thought incompatible. U.S. Patent No. 4,881,989 discloses an Fe-based soft magnetic alloy with ultrafine crystal grains having both high saturation magnetic flux density Bs and high relative permeability µ. This Fe-based alloy having an average grain size of 50 nm (500Å) or less is produced through a crystallization process after it is quenched rapidly into an amorphous state. This Fe-based alloy with ultrafine crystal grains has good corrosion resistance to some extent because it contains Nb, etc. When this alloy is used for magnetic cores, it is preferably coated with an oxidation layer. The corrosion resistance of this Fe-based alloy, however, may not be sufficient depending on surroundings in which it is used.

JP-A-4-21746 discloses ultrafine-grain iron alloys having asymmetric magnetization curve, consisting of (Fe₁₋ₐMₐ)_{100-x-y-z-α-β-γ-}AₓSi_{y}B_{z}M¹_{α}M²_{β}X_{γ} at.% and containing ≥ 50 % fine crystals with an average diameter of ≤ 1000 µm.

JP-A-4-9401 discloses powder manufactured from melt-quenched iron alloy having soft magnetic properties and being resistant to corrosion, which alloy contains, by at.%, 15-18 Si, 5-9 B, 1-4 Cr, 0.1-3 Cu, and 2-10 Nb, Mo, Ta and/or W. Said powder is provided with a dense oxide film.

EP-A-430 085 discloses a magnetic alloy with ultrafine crystal grains having an At.% composition of Fe_{100-x-y-}MₓB_{y}, wherein M is at least one of Ti, Zr, Hf, V, Nb, Mo, Ta, Cr, W and Mn, 4 ≤ x ≤ 15, 2 ≤ y ≤ 25 and 7 ≤ x + y ≤ 35, and optionally of (Si, Ge, P, Ga etc.) and/or (Au, Co, Ni etc.), at least 50 % of the alloy structure being occupied by crystal grains having an average grain size of 500 Å or less.

The same alloy structure is disclosed by EP-A-429 022 for a magnetic alloy having an At.% composition of Co_{100-x-y-z-a-b}FeₐMₓB_{y}X_{z}T_{b}, wherein M is at least one of Ti, Zr, Hf, V, Nb, Mo, Ta, Cr, W and Mn, X is at least one of Si, Ge, P, Ga, Al and N, T is at least one of Cu, Ag, Au, platinum group elements, Ni, Sn, Be, Mg, Ca, Sr and Ba, 0 < a ≤ 30, 2 ≤ x ≤ 15, 10 ≤ y ≤ 25, 0 ≤ z ≤ 10, 0 < b ≤ 10, and 12 < x + y + z + b ≤ 35.

JP-A-2 159 315 discloses a heat treatment in grain refinement of a soft magnetic iron alloy containing Cu and Nb, W, Ta, Zr, Hf and/or Mo to obtain a microstructure containing ≥ 50 % superfine grains and showing a magnetic permeability (at 1 kHz) of 92000 - 118 000.

JP-A-1 287 250 discloses heat-resistant soft magnetic iron alloys having a composition of (Fe₁₋ₐMₐ)_{100-x-y-z-α-δ}CuₓSi_{y}B_{z}M'_{α}T_{δ}, where M is Co and/or Ni, M' is Nb, W, Ta, Zr, Hf, Ti and/or Mo; T is C, P, O, S and/or N and a ≤ 0.1, x = 0.1 - 3, y ≤ 30, z ≤ 25, y + z = 5 - 30, α ≤ 30, and δ ≤ 0.15, and having ≥ 50 % fine grains of average size ≤ 1000 Å in the structure.

JP-A-3-60105 discloses a soft magnetic cobalt alloy film having a composition of CoₓPd_{y}M_{z}C_{w} (M = Ti, Zr, Hf, V, Nb, Ta, Mo and/or W; 50 ≤ x ≤ 96; 0.1 ≤ y ≤ 20; 2 ≤ z ≤ 25; 0.5 ≤ w ≤ 25; x+y+z+w = 100), wherein M carbide crystal phases partially exist.

JP-A-3-215 650 discloses iron alloys having perminvar characteristics which contain Fe; Cu, Ag and/or Au; Nb, W, Ta, Zr, Hf, Ti, V, Mn, Cr and/or Mo, wherein ≥ 50 % of the texture consist of ultrafine crystal grains ≤ 1000 Å in average grain diameter.

### OBJECT AND SUMMARY OF THE INVENTION

Accordingly, an object of the present invention is to provide an alloy with ultrafine crystal grains having improved corrosion resistance.

As a result of an intense research for solving the above problems, the inventors have found that the alloy having a specific surface layer shows extremely improved corrosion resistance.

Said object is achieved, according to the present invention, by an alloy as claimed in claim 1 which alloy shows excellent corrosion resistance.

Further advantageous features are claimed in claims 2 - 6.

### BRIEF DESCRIPTION OF THE DRAWING

Fig. 1 is a graph showing the Is spectra of O in the surface layers of the fine crystalline alloys of the present invention;
Fig. 2 is a graph showing the 2p_{3/2} spectra of Fe in the surface layers of the fine crystalline alloys of the present invention;
Fig. 3 is a graph showing the 2p spectra of Si in the surface layers of the fine crystalline alloys of the present invention;
Fig. 4 is a graph showing the 1s spectra of O in the surface layers of the fine crystalline alloys of the present invention;
Fig. 5 is a graph showing the 2p_{3/2} spectra of Fe in the surface layers of the fine crystalline alloys of the present invention;
Fig. 6 is a graph showing the 2p spectra of Si in the surface layers of the fine crystalline alloys of the present invention; and
Fig. 7 is a graph showing the 1s spectra of O in the surface layers of the fine crystalline alloys of the present invention formed by anodizing.

### DETAILED DESCRIPTION OF THE INVENTION

The present invention will be described in detail below.

The surface layers of the fine crystalline alloy according to the present invention can be identified by X-ray photoelectron spectroscopy ESCA. ESCA is a chemical element analysis comprising the steps of applying X-ray to a sample and detecting photoelectrons emitted from the sample for identifying chemical bonds of elements by chemical shift values of bond energies. In the description of the present invention, the presence of hydroxides is confirmed by observing peaks attributed to hydroxides in an ESCA spectrum. Same is true of oxide components. More specific understanding can be attained by examples described below.

As is shown by Examples below, when the fine crystalline alloys contain larger amounts of hydroxide components than those of oxide components in the surface layers, they show excellent corrosion resistance. In this case, when the surface layers are thin in the Fe-based alloys, Fe⁰ under the surface layers (inside alloys) is strongly detected. On the other hand, Fe²⁺ and Fe³⁺ are observed in the surface layers. Furthermore, in the case of the fine crystalline alloys containing Si, they show excellent corrosion resistance if the surface layers contain Si⁴⁺. When Si⁴⁺ exists in the form of SiO_{2,} the fine crystalline alloys show excellent corrosion resistance in most cases.

When the surface layers of the fine crystalline alloys contain oxides of at least one element selected from the group consisting of Ta, Nb and Cr, they have particularly excellent corrosion resistance. In that case, these elements are not necessarily in the state of complete oxides but usually are in an intermediate state between oxides and metals. When they contain at least one element selected from the group consisting of Zr, Hf and W, their corrosion resistance in an alkaline environment is improved.

When the average grain size is as small as 50 nm (500Å) or less in the fine crystalline alloy, corrosion resistance is further improved, and magnetic and mechanical properties are also improved to a level preferable for practical applications. Particularly desirable average grain size is from 2 nm (20Å) to 20 nm (200Å) since the structure of the fine crystalline alloy is fine and uniform in this average grain size range.

The fine crystalline alloys to which the present invention is applicable have a composition represented by the general formula:

M_{100-x-y-z-α-β-γ} AₓSi_{y}B_{z}M'_{α}M"_{β}X_{γ} (atomic %)

wherein M represents at least one element selected from the group consisting of Fe, Co and Ni; A represents at least one element selected from the group consisting of Cu, Ag and Au; M' represents at least one element selected from the group consisting of Nb, Mo, Ta, Ti, Zr, Hf, V, Cr and W; M" represents at least one element selected from the group consisting of Mn, Al, platinum group elements, Sc, Y, rare earth elements, Zn, Sn and Re; X represents at least one element selected from the group consisting of C, Ge, P, Ga, Sb, In, Be and As, 0≤x≤10, 0≤y≤30, 0≤z≤25, 0≤y+z≤30, 1≤α≤20, 0≤β≤20, and 0≤γ≤20.

The element M is at least one ferromagnetic element selected from the group consisting of Fe, Co and Ni.

The element A representing at least one element selected from the group consisting of Cu, Ag and Au, which effectively makes the alloy structure finer in cooperation with the element M'.

The element M' representing at least one element selected from the group consisting of Nb, Mo, Ta, Ti, Zr, Hf, V, Cr and W makes the alloy structure considerably finer in cooperation with the element A. Among the elements mentioned above, at least one element selected from the group consisting of Nb, Ta and Cr makes it easier to provide the surface layer with improved corrosion resistance.

Si and B are effective elements for making the alloys amorphous, for improving magnetic properties, and for making the alloy structure finer. Si functions to improve the corrosion resistance of the surface layers of the fine crystalline alloys, and if Si exists in the form of SiO₂ in the surface layers, their corrosion resistance is extremely improved.

The element M'' representing at least one element selected from the group consisting of Mn, Al, platinum group elements, Sc, Y, rare earth elements, Zn, Sn and Re is effective for improving corrosion resistance and for controlling magnetic properties.

The element X representing at least one element selected from the group consisting of C, Ge, P, Ga, Sb, In, N, Be and As is effective for making the alloy structure amorphous and for controlling magnetic properties.

With the above-mentioned surface layers, the corrosion rate of the fine crystalline alloys in a 0.1-kmol·m⁻³ NaCl aqueous solution can be reduced to as small as 1 × 10⁻⁸ kg·m⁻²·s⁻¹ or less.

The fine crystalline alloys of the present invention can be produced by the steps of preparing amorphous alloys by a liquid quenching method such as a single roll method, a double roll method, a rotating liquid spinning method, etc., or by a gas phase quenching method such as a sputtering method, a vapor deposition method, etc., and conducting a heat treatment on the amorphous alloys for turning at least 50% of the alloy structures into ultrafine crystal grains. Though the balance of the alloy structures is usually amorphous, the present invention includes alloys having alloy structures practically consisting of ultrafine crystal phase. The fine crystalline alloys of the present invention can also be produced by the steps of forming amorphous alloy layers in surface portions of alloys by applying laser rays thereto, and conducting a heat treatment thereon. The powdery alloys of the present invention can be produced by conducting a heat treatment on atomized amorphous alloys.

In the processes having a heat treatment step, the heat treatment is preferably conducted at 450°C-800°C. When the heat treatment temperature is lower than 450°C, fine crystallization is difficult even though the heat treatment is conducted for a long period of time. On the other hand, when it exceeds 800°C, the crystal grains grow excessively, failing to obtain the desired ultrafine crystal grains. The preferred heat treatment temperature is 500-700°C. Incidentally, the heat treatment time is generally 1 minute to 200 hours, preferably 5 minutes to 24 hours. The heat treatment temperatures and time may be determined within the above ranges depending upon the compositions of the alloys. The above heat treatment may be conducted in an inert atmosphere.

The heat treatment of the alloys of the present invention can be conducted in a magnetic field. When a magnetic field is applied in one direction, a magnetic anisotropy in one direction can be given to the resulting heat-treated alloys. Also, by conducting the heat treatment in a rotating magnetic field, further improvement in soft magnetic properties can be achieved. In addition, the heat treatment for fine crystallization can be followed by a heat treatment in a magnetic field.

Alternatively, the alloys of the present invention with ultrafine crystal grains can be directly produced without experiencing an amorphous phase by controlling quenching conditions.

It is possible to provide the fine crystalline alloys of the present invention with surface layers containing hydroxide components by a heat treatment in an inert atmosphere containing oxygen and steam, or by anode oxidation before or after the crystallization heat treatment.

In the case of the heat treatment in an inert gas atmosphere containing oxygen and steam, the inert atmosphere should contain 0,1 - 3 volume % of oxygen and 10 - 100 ppm of steam. The preferred oxygen content is about 0,5 volume %, and the preferred steam content is 20 - 50 ppm.

The heat treatment for forming the surface layers is preferably conducted at 250-700°C. When the heat treatment temperature is lower than 250°C, surface layers with good corrosion resistance cannot be obtained. On the other hand, when it exceeds 700°C, crystal grains become too large in the resultant surface layers.

The heat treatment for forming the surface layers may be conducted at the same time as the heat treatment for fine crystallization. In this case, the heat treatment may be conducted at 450-700°C for 10 minutes to 24 hours in an inert atmosphere containing oxygen and steam.

The present invention includes fine crystalline alloys having the above-mentioned surface layers formed by sputtering, vapor deposition, CVD etc.

The present invention will be explained in further detail by way of the following Examples, without intending to restrict the scope of the present invention.

### Example 1

Three kinds of alloy melts having the following compositions:
- Comparative Example 1:: Fe_{bal.}Cu₁Si_{13.5}B_{9,} (Sample 1)
- Sample 2:: Fe_{bal.}Cu₁Nb₅Si_{13.5}B₉, and
- Sample 3:: Fe_{bal.}Cu₁Nb₇Si₁₆B₉
were rapidly quenched by a single roll method to produce thin amorphous alloy ribbons of 5 mm in width and about 18 µm in thickness. A heat treatment was then conducted to the alloy ribbons at 570°C in a nitrogen gas atmosphere containing 0.5 volume % of oxygen and 30 ppm of steam for 1 hour. The heat-treated alloys had crystallized structures, 90% or more of which were occupied by ultrafine crystal grains of an average grain size of 10 nm (100Å).

The surface layers of the fine crystalline alloys were then observed by ESCA. Procedures and conditions of this analysis were as follows: Each sample cut into a size of 4 mm × 4 mm for analysis was fixed to a probe with a double-sided adhesive tape of conductive carbon. Mg-Kα-ray was used for an excitation X-ray, which was generated at 5 kV and 30 mA. The analysis was done at a reduced pressure of 2.7 x 10⁻⁷hPa (2 × 10⁻⁷ Torr) or lower.

The corrosion rates of the fine crystalline alloys were also measured in a 0.1-kmol·m⁻³ NaCl aqueous solution. The measured corrosion rates of the fine crystalline alloys were as follows:
- Comparative Example 1:: 2.02 × 10⁻⁸ kg·m⁻²·s⁻¹,
- Sample 2:: 8.27 × 10⁻¹¹ kg·m⁻²·s⁻¹, and
- Sample 3:: almost 0 kg·m⁻²·s⁻¹.

The 1s spectra of O in the surface layers of the above fine crystalline alloys are shown in Fig. 1. In the spectra of Samples 2 and 3 excellent in corrosion resistance, the peaks attributed to the hydroxides M(OH)_{y}, wherein M represents a transition metal and y represents a valency of M, were as large as 65% or more, while those attributed to MOₓ, wherein x represents one-half of the valency of M, were as small as 35% or less. This fact indicates that the fine crystalline alloys having the surface layers in which the total proportion of the peaks attributed to the hydroxides M(OH)_{y} are as large as 65% or more based on the integrated value of the entire spectrum of M have better corrosion resistance.

The 2p_{3/2} spectra of Fe in the surface layers of these fine crystalline alloys are shown in Fig. 2. In all of the fine crystalline alloys, the peaks attributed to Fe²⁺ and Fe³⁺ were observed, indicating that the surface layers contained Fe₂O₃, etc. Furthermore, a peak corresponding to FeOOH was also observed in the surface layers. The spectra of Fe⁰ were observed in the surface layers of Samples 2 and 3 excellent in corrosion resistance. It was, therefore, confirmed that the surface layers were so thin that Fe under the surface layers could be detected.

The 2p spectra of Si in the surface layers of these fine crystalline alloys are shown in Fig. 3. In the case of Samples 2 and 3 having excellent corrosion resistance, Si⁴⁺ (identified as SiO₂ in Fig. 3) was mainly observed, while components in an intermediate oxidation state between Si⁰ and Si⁴⁺ (SiO₂) were not observed. The corrosion resistance of the fine crystalline alloys tends to be improved as the amount of Si⁴⁺ (SiO₂) increases.

### Example 2

Four kinds of alloy melts having the following compositions:
- Comparative Example 4:: Fe_{bal.}Cu₁Si_{13.5}B_{9,} (Sample 4)
- Sample 5:: Fe_{bal.}Cu₁Nb₅Si_{13.5}B₉,
- Sample 6:: Fe_{bal.}Cu₁Ta₅Si_{13.5}B₉, and
- Sample 7:: Fe_{bal.}Cu₁Ti₅Si_{13.5}B₉
were rapidly quenched by a single roll method to produce thin amorphous alloy ribbons of 5 mm in width and about 18 µm in thickness. A heat treatment was then conducted to the alloy ribbons at 590°C in a nitrogen gas atmosphere containing 0.5% of oxygen and 30 ppm of steam for 1 hour. The heat-treated alloys had crystallized structures, 90% or more of which were occupied by ultrafine crystal grains of an average grain size of 11 nm (110Å).

The surface layers of the fine crystalline alloys were observed by X-ray photoelectron spectroscopy ESCA in the same way as described in Example 1. The corrosion rates of the fine crystalline alloys were measured in a 0.1-kmol·m⁻³ NaCl aqueous solution. The measured corrosion rates of the fine crystalline alloys were as follows:
- Comparative Example 4:: 2.02 × 10⁻⁸ kg·m⁻²·s⁻¹,
- Sample 5:: 8.27 × 10⁻¹¹ kg·m⁻²·s⁻¹,
- Sample 6:: 8.24 × 10⁻¹¹ kg·m⁻²·s⁻¹, and
- Sample 7:: 1.01 × 10⁻⁹ kg·m⁻²·s⁻¹.

The 1s spectra of O in the surface layers of the above fine crystalline alloys are shown in Fig. 4. In the spectra of Samples 5 and 6 excellent in corrosion resistance, the peaks attributed to the hydroxides M(OH)_{y} were as large as 65% or more, while those attributed to MOₓ were as small as 35% or less. This fact indicates that the fine crystalline alloys having the surface layers in which the total proportion of the peaks attributed to the hydroxides M(OH)_{y} are as large as 65% or more based on the integrated value of the entire spectrum of M have better corrosion resistance.

The 2p_{3/2} spectra of Fe in the surface layers of these fine crystalline alloys are shown in Fig. 5. The spectra of Fe⁰ were observed in the surface layers of Samples 5 and 6 excellent in corrosion resistance. It was, therefore, confirmed that the surface layers were so thin that Fe under the surface layers could be detected. The peaks attributed to Fe²⁺ and Fe³⁺ were also observed, indicating that the surface layers contained Fe₂O₃, etc. Furthermore, a peak attributed to FeOOH was observed.

The 2p spectra of Si in the surface layers of these fine crystalline alloys are shown in Fig. 6. In the case of Samples 5 and 6 having excellent corrosion resistance, Si⁴⁺ (identified as SiO₂ in Fig. 6) was mainly observed, while components in an intermediate oxidation state between Si⁰ and Si⁴⁺ (SiO₂) were not observed. The corrosion resistance of the fine crystalline alloys tends to be improved as the amount of Si⁴⁺ (SiO₂) increases.

### Example 3

Three kinds of alloy melts having the following compositions:
- Sample 8:: Fe_{bal.}Cu₁Nb₅Si_{13.5}B₉,
- Sample 9:: Fe_{bal.}Cu₁Ta₅Si_{13.5}B₉, and
- Sample 10:: Fe_{bal.}Cu₁Ti₅Si_{13.5}B₉
were rapidly quenched by a single roll method to produce thin amorphous alloy ribbons of 5 mm in width and about 18 µm in thickness. A heat treatment was then conducted on the alloy ribbons at 590°C in a nitrogen gas atmosphere containing 0.001 volume % of oxygen and 10 ppm of steam for 1 hour. The heat-treated alloys had crystallized structures, 90% or more of which were occupied by ultrafine crystal grains of an average grain size of 10 nm (100Å). After the heat treatment, the fine crystalline alloys were anodized to form surface oxide layers under the following conditions:
- Sample 8: In 0.1-kmol·m⁻³ NaCl aqueous solution at 298 K at -0.2 V (vs. Ag/AgCl) for 1 hour,
- Sample 9: In 0.1-kmol·m⁻³ NaCl aqueous solution at 298 K at +0.3 V (vs. Ag/AgCl) for 1 hour, and
- Sample 10: In 0.1-kmol·m⁻³ NaCl aqueous solution at 298 K at -0.2 V (vs. Ag/AgCl) for 1 hour.

The 1s spectra of O in the surface layers of the above fine crystalline alloys are shown in Fig. 7. In the spectra of Samples 8 and 9 having excellent corrosion resistance, the peaks attributed to the hydroxides M(OH)_{y} were as large as 65% or more, while those attributed to MOₓ were as small as 35% or less. This fact indicates that the fine crystalline alloys having the surface layers in which the total proportion of the peaks attributed to the hydroxides M(OH)_{y} are as large as 65% or more based on the integrated value of the entire spectrum of M have better corrosion resistance.

### Example 4

Alloy melts having compositions listed in Table 1 were rapidly quenched by a single roll method to produce thin amorphous alloy ribbons of 5 mm in width and about 18 µm in thickness. A heat treatment was then conducted on the alloy ribbons at 570°C in a nitrogen gas atmosphere containing 0.5% of oxygen and 30 ppm of steam for 1 hour. The heat-treated alloys had crystallized structures, 90% or more of which were occupied by ultrafine crystal grains of an average grain size of 10 nm (100Å).

The surface layers of the fine crystalline alloys were then observed by ESCA in the same way as described in Example 1. The ratio of hydroxide components to oxide components and the proportion of Si⁴⁺ bonds in the surface layers were determined from the ratio in intensity of a peak attributed to each bond to the integrated spectrum intensity of the element. Here, the 1s spectrum of O was assumed to be attributed mainly to four components derived from (1) H₂O adsorbed onto the surfaces of the fine crystalline alloys, derived from (2) hydroxides, derived from (3) SiO₂ formed by the oxidation of Si, one of alloy elements, and derived from (4) oxides of Fe, etc., one of alloy elements. Each bond state of O was determined by comparing the observed 1s spectrum of O with a spectrum synthesized from spectra of each bond by approximation of the Gauss-Lorenz mixed distribution.

The ratio of the hydroxide components to the oxide components was defined as a ratio of (a) a proportion of peaks attributed to the hydroxide components in the integrated spectrum of O to (b) a proportion of peaks attributed to the oxide components in the integrated spectrum of O. Incidentally, it is difficult to completely separate each spectrum since peaks in the 1s spectrum of O attributed to the hydroxides components and Si⁴⁺ (SiO₂) are close to each other. Thus, the intensity of a peak attributed to MOx in the 1s spectrum of O was presumed from the intensity of a peak attributed to Si⁴⁺ (SiO₂) in the 2p spectrum of Si.

The corrosion rates of the fine crystalline alloys were also measured in 0.1-kmol·m⁻³ NaCl aqueous solution like Example 1. The measured corrosion rates, the ratios of hydroxide components to oxide components, and the ratios of Si⁴⁺ are listed in Tables 1 and 2. In the case of the fine crystalline alloys containing Fe, the surface layers contained compounds of both Fe²⁺ and Fe³⁺.

**Table 1**

| Sample No.⁽¹⁾ | Composition (atomic %) | Corrosion Rate⁽²⁾ | Hydroxide/Oxide⁽³⁾ | Ratio of Si⁴⁺(%) |
|---|---|---|---|---|
| 11 | Fe_{bal.}Cu₁Si_{13.5}B₉Nb₅ | 8.27 x 10⁻¹¹ | 108 | 93 |
| 12 | Fe_{bal.}Cu₁Si_{13.5}B₉Ta₅ | 8.24 x 10⁻¹¹ | 246 | 91 |
| 13 | Fe_{bal.}Cu₁Si_{13.5}B₉Cr₅ | 8.27 x 10⁻¹¹ | 201 | 97 |
| 14 | Fe_{bal.}Cu₁Si_{13.5}B₉Zr₅ | 5.95 x 10⁻¹¹ | 105 | 91 |
| 15 | Fe_{bal.}Cu₁Si_{13.5}B₉Hf₅ | 3.3 x 10⁻¹⁰ | 98 | 90 |
| 16 | Fe_{bal.}Cu₁Si_{13.5}B₉Nb₅W₂ | 8.47 x 10⁻¹¹ | 110 | 92 |
| 17 | Fe_{bal.}Cu₁Si_{13.5}B₉Nb₅Hf₅ | 5.12 x 10⁻¹¹ | 208 | 94 |
| 18 | Fe_{bal.}Cu₁Si_{13.5}B₉Nb₇ | Almost 0 | 100 | 94 |
| 19 | Co_{bal.}Cu₁Si_{13.5}B₉Nb₅Zr₁ | 5.25 x 10⁻¹¹ | 125 | 95 |
| 20 | Ni_{bal.}Cu₁Si_{13.5}B₉Nb₅Cr₅ | 4.65 x 10⁻¹¹ | 140 | 96 |
| 21 | Fe_{bal.}Au₁Si₁₀B₆Zr₇ | 8.95 x 10⁻¹¹ | 97 | 86 |
| 22 | Fe_{bal.}Cu₁Si_{13.5}B₉Nb₅Al₃ | 7.89 x 10⁻¹¹ | 115 | 95 |
| 23 | Fe_{bal.}Cu₁Si_{13.5}B₉Nb₅Ge₃ | 8.86 x 10⁻¹¹ | 98 | 90 |
| 24 | Fe_{bal.}Cu₁Si_{13.5}B₉Nb₅Ga₁ | 9.26 x 10⁻¹¹ | 96 | 88 |
| 25 | Fe_{bal.}Cu₁Si_{13.5}B₉Nb₅P₁ | 8.36 x 10⁻¹¹ | 92 | 87 |
| 26 | Fe_{bal.}Cu₁Si_{13.5}B₉Nb₅Ru₂ | 7.29 x 10⁻¹¹ | 120 | 89 |
| 27 | Fe_{bal.}Cu₁Si_{13.5}B₉Nb₅Pd₂ | 8.52 x 10⁻¹¹ | 101 | 88 |
| 28 | Fe_{bal.}Cu₁Si_{13.5}B₉Nb₅Pt₂ | 7.94 x 10⁻¹¹ | 99 | 92 |
| 29 | Fe_{bal.}Cu₁Si_{13.5}B₉Nb₅C_{0.2} | 8.78 x 10⁻¹¹ | 118 | 86 |
| 30 | Fe_{bal.}Cu₁Si_{13.5}B₉Nb₅Mo₂ | 8.12 x 10⁻¹¹ | 120 | 88 |
| 31 | Fe_{bal.}Cu₁Si_{13.5}B₉Nb₅Mn₅ | 9.46 x 10⁻¹¹ | 105 | 89 |

| | | | | |
|---|---|---|---|---|
| Note: (1) Examples of the present invention. | | | | |
| (2) Unit is kg·m⁻²·s⁻¹. | | | | |
| (3) Ratio of hydroxides to oxides (%). | | | | |

**Table 2**

| Sample No.⁽¹⁾ | Composition (atomic %) | Corrosion Rate⁽²⁾ | Hydroxide/Oxide⁽³⁾ | Ratio of Si⁴⁺(%) |
|---|---|---|---|---|
| 32 | Fe_{bal.}Cu₁Si_{13.5}B₉ | 2.02 x 10⁻⁸ | 64 | 55 |
| 33 | Fe_{bal.}Cu₁Si_{13.5}B₉Ti₁ | 1.58 x 10⁻⁸ | 63 | 62 |
| 34 | Fe_{bal.}Cu₁Si_{13.5}B₉W₃ | 2.04 x 10⁻⁸ | 62 | 52 |
| 35 | Fe_{bal.}Cu₁Si_{13.5}B₉Mn₅ | 2.28 x 10⁻⁸ | 60 | 51 |

| | | | | |
|---|---|---|---|---|
| Note: (1) Comparative Examples. | | | | |
| (2) Unit is kg·m⁻²·s⁻¹. | | | | |
| (3) Ratio of hydroxides to oxides (%). | | | | |

It is clear from Tables 1 and 2 that the ratios (hydroxide components to oxide components) was 65% or more in the surface layers of the fine crystalline alloys, the fine crystalline alloys showed excellent corrosion resistance. Particularly when the surface layers contain Si⁴⁺ (SiO₂), and when the ratio of Si⁴⁺ peaks to the integrated value of the entire 2p spectrum of Si is more than 55%, the fine crystalline alloys show excellent corrosion resistance (very small corrosion rate). Fine crystalline alloys containing Ta, Nb and Cr have particularly excellent resistance owing to oxides of these elements.

The present invention can provide fine crystalline alloys having excellent corrosion resistance.

## Claims

1. An alloy with ultrafine crystal grains excellent in corrosion resistance, at least 50 % of the alloy structure being occupied by ultrafine crystal grains having an average grain size of 50 nm (500 Å) or less, said alloy having a composition represented by the general formula:
M_{100-x-y-z-α-β-γ} AₓSi_{y}B_{z}M'_{α}M"_{β}X_{γ} (atomic %),
wherein M represents at least one element selected from the group consisting of Fe, Co and Ni; A represents at least one element selected from the group consisting of Cu, Ag and Au; M' represents at least one element selected from the group consisting of Nb, Mo, Ta, Ti, Zr, Hf, V, Cr and W; M" represents at least one element selected from the group consisting of Mn, Al, platinum group elements, Sc, Y, rare earth elements, Zn, Sn and Re; X represents at least one element selected from the group consisting of C, Ge, P, Ga, Sb, In, Be and As, 0 ≤ x ≤ 10, 0 ≤ y ≤ 30, 0 ≤ z ≤ 25, 0 ≤ y+z ≤ 30, 1 ≤ α ≤ 20, 0 ≤ β ≤ 20, and 0 ≤ γ ≤ 20,
said alloy having a surface layer containing hydroxide components, and said hydroxide components are in a total proportion of 65 % or more based on oxide components.

2. The alloy according to claim 1, wherein said alloy is an Fe-based alloy and has a surface layer containing compounds of Fe²⁺ and Fe³⁺, and wherein Fe⁰ spectrum is observed in said alloy by X-ray photoelectron spectroscopy.

3. The alloy according to claim 1 or 2, wherein said alloy contains Si and has a surface layer containing a compound of Si⁴⁺, and wherein the ratio of Si⁴⁺ peaks to an integrated value of entire 2p spectrum of Si is more than 55% by X-ray photoelectron spectroscopy.

4. The alloy according to any one of claims 1-3, wherein said surface layer contains an oxide of at least one element selected from the group consisting of Ta, Nb and Cr.

5. The alloy according to any one of claims 1-3, wherein said surface layer contains an oxide of at least one element selected from the group consisting of Zr, Hf and W.

6. The alloy according to any one of claims 1-5, wherein the corrosion rate of said alloy in a 0.1-kmol·m⁻³ NaCl aqueous solution is 1 × 10⁻⁸ kg·m⁻²·s⁻¹ or less.

## Patentansprüche

1. Legierung mit ultrafeinen Kristallkörnern hervorragender Korrosionsbeständigkeit, wobei wenigstens 50 % des Legierungsgefüges von ultrafeinen Kristallkörnern einer Durchschnittskorngröße von 50 nm (500 Å) oder weniger eingenommen werden, welche Legierung eine durch die allgemeine Formel
M_{100-x-y-z-α-β-γ}AₓSi_{y}B_{z}M'_{α}M"_{β}X_{γ} (At.%),
dargestellte Zusammensetzung hat, worin M wenigstens ein aus der aus Fe, Co und Ni bestehenden Gruppe gewähltes Element bedeutet; A wenigstens ein aus der aus Cu, Ag und Au bestehenden Gruppe gewähltes Element bedeutet; M' wenigstens ein aus der aus Nb, Mo, Ta, Ti, Zr, Hf, V, Cr und W bestehenden Gruppe gewähltes Element bedeutet; M" wenigstens ein aus der aus Mn, Al, Platingruppenelementen, Sc, Y, Seltenerdelementen, Zn, Sn und Re bestehenden Gruppe gewähltes Element bedeutet; X wenigstens ein aus der aus C, Ge, P, Ga, Sb, In, Be und As bestehenden Gruppe gewähltes Element bedeutet; 0 ≤ x ≤ 10, 0 ≤ y ≤ 30, 0 ≤ z ≤ 25, 0 ≤ y+z ≤ 30, 1 ≤ α ≤ 20, 0 ≤ β ≤ 20 und 0 ≤ γ ≤ 20,
welche Legierung eine Hydroxidbestandteile enthaltende Oberflächenschicht aufweist, wobei die Hydroxidbestandteile im Gesamtanteil von 65 % oder mehr auf Basis von Oxidbestandteilen sind.

2. Legierung nach Anspruch 1,
wobei die Legierung eine Fe-Basislegierung ist und eine Fe²⁺- und Fe³⁺-Verbindungen enthaltende Oberflächenschicht hat und wobei ein Fe⁰-Spektrum in der Legierung durch Röntgenstrahlen-Photoelektronenspektroskopie beobachtet wird.

3. Legierung nach Anspruch 1 oder 2,
wobei die Legierung Si enthält und eine eine Si⁴⁺-Verbindung enthaltende Oberflächenschicht hat und wobei das Verhältnis von Si⁴⁺-Spitzen zu einem integrierten Wert des gesamten 2p-Spektrums von Si mehr als 55 % durch Röntgenstrahlen-Photoelektronenspektroskopie ist.

4. Legierung nach irgendeinem der Ansprüche 1-3,
wobei die Oberflächenschicht ein Oxid wenigstens eines aus der aus Ta, Nb und Cr bestehenden Gruppe gewählten Elements enthält.

5. Legierung nach irgendeinem der Ansprüche 1-3,
wobei die Oberflächenschicht ein Oxid wenigstens eines aus der aus Zr, Hf und W bestehenden Gruppe gewählten Elements enthält.

6. Legierung nach irgendeinem der Ansprüche 1-5,
wobei der Korrosionsgrad der Legierung in einer wässerigen 0,1 kmol·m⁻³ NaCl-Lösung 1 x 10⁻⁸ kg·m⁻²·s⁻¹ oder weniger ist.

## Revendications

1. Alliage à grains cristallins ultrafins ayant une excellente résistance à la corrosion, au moins 50 % de la structure d'alliage étant occupés par des grains cristallins ultrafins ayant une granulométrie moyenne de 50 nm (500 Å) ou moins, ledit alliage ayant une composition représentée par la formule générale suivante :
M_{100-x-y-z-α-β-Γ-}AₓSi_{y}B_{z}M'_{α}M"_{β}X_{Γ} (en pourcentages atomiques),
caractérisé en ce que M représente au moins un élément choisi dans l'ensemble constitué par Fe, Co et Ni ; A représente au moins un élément choisi dans l'ensemble constitué par Cu, Ag et Au ; M' représente au moins un élément choisi dans l'ensemble constitué par Nb, Mo, Ta, Ti, Zr, Hf, V, Cr et W ; M" représente au moins un élément choisi dans l'ensemble constitué par Mn, Al, les éléments du groupe du platine, Sc, Y, les éléments des terres rares, Zn, Sn et Re ; X représente au moins un élément choisi dans l'ensemble constitué par C, Ge, P, Ga, Sb, In, Be et As, 0 ≤ x ≤ 10, 0 ≤ y ≤ 30, 0 ≤ z ≤ 25, 0 ≤ y + z ≤ 30, 1 ≤ α ≤ 20, 0 ≤ β ≤ 20, et 0 ≤ Γ ≤ 20,
ledit alliage ayant une couche superficielle contenant des composants de type hydroxyde, et lesdits composants de type hydroxyde sont présents en une proportion totale de 65 % ou plus par rapport aux composants de type oxyde.

2. Alliage selon la revendication 1, caractérisé en ce que ledit alliage est un alliage à base de Fe et a une couche superficielle contenant des composés de Fe²⁺ et Fe³⁺, et dans lequel un spectre de Fe⁰ est observé dans ledit alliage par spectroscopie photoélectronique aux rayons X.

3. Alliage selon l'une des revendications 1 ou 2, caractérisé en ce que ledit alliage contient du Si et a une couche superficielle contenant un composé de Si⁴⁺, et en ce que le rapport des pics de Si⁴⁺ à une valeur intégrée du spectre 2p complet de Si est supérieur à 55 % par spectroscopie photoélectronique aux rayons X.

4. Alliage selon l'une quelconque des revendications 1 à 3, caractérisé en ce que ladite couche superficielle contient un oxyde d'au moins un élément choisi dans l'ensemble constitué par Ta, Nb et Cr.

5. Alliage selon l'une quelconque des revendications 1 à 3, caractérisé en ce que ladite couche superficielle contient un oxyde d'au moins un élément choisi dans l'ensemble constitué par Zr, Hf et W.

6. Alliage selon l'une quelconque des revendications 1 à 5, caractérisé en ce que la vitesse de corrosion dudit alliage dans une solution aqueuse à 0,1 kmol.m⁻³ de NaCl est de 1 x 10⁻⁸ kg.m⁻².s⁻¹ ou moins.
